

## 1

3,514,292

## SILVER HALIDE EMULSION CONTAINING PYRROLIDINE PROLINE OR HYDROXYPROLINE SENSITIZERS

Raymond Joseph Le Strange, Middletown, N.J., assignor to E. I. du Pont de Nemours and Company, Wilmington, Del., a corporation of Delaware

No Drawing. Filed May 19, 1967, Ser. No. 639,655  
Int. Cl. G03c 1/28

U.S. CL. 96—107

7 Claims

## ABSTRACT OF THE DISCLOSURE

A gelatino silver halide emulsion of increased sensitivity to radiation is obtained by adding a sensitizing amount of pyrrolidine, 2-pyrrolidine carboxylic acid (proline), or 4-hydroxy-2-pyrrolidine carboxylic acid (hydroxyproline).

It has long been known that silver halide photographic emulsions may be sensitized by adding degradation products of various animal and vegetable materials, these degradation products being obtained by electrodialysis (U.S. Pat. 1,667,589), alkaline or alkaline fermentative hydrolysis and simultaneous partial oxidation (U.S. Pat. 1,719,711), acid hydrolysis (British Pat. 259,926), or acid hydrolysis and simultaneous partial oxidation (U.S. Pat. 1,815,983). The above processes yield degradation products rich in varying concentrations of many, inseparable constituents, ranging from higher molecular weight polypeptide combinations of amino acids to lower molecular weight polypeptide fragments, and may even contain carbohydrates, aldehydes and other organic acids which sensitometrically affect photographic emulsions.

Experimental data has been reported where various individual proteins, such as tyrosine, alanine, proline, hydroxyproline, leucine, cystine and others were added to ammoniacal, positive, silver bromide emulsions, and the sensitometric effects were observed. The proteins were added in an amount proportional to their concentration in gelatin. The results reported that while proline and hydroxyproline retard the appearance of fog in the developed emulsion, they reduce the speed of the emulsion.

Recent trends toward improved processing characteristics, such as shorter drying times and lower residual thiosulfate content, have resulted in reducing the amount of binder, e.g. gelatin, contained in the emulsion. This reduction in binder content in many instances is accompanied by a significant loss in sensitivity.

This invention relates to an improved gelatino silver halide emulsion wherein pyrrolidine, 2-pyrrolidine carboxylic acid, or 4-hydroxy-2-pyrrolidine carboxylic acid is added, in the amount of from 0.13 to 3.34 grams per mole of silver, to increase sensitivity to radiation without increasing fog.

The addition of these compounds in their pure form allows for controlled use and reproducible sensitization. In addition, the compounds of this invention provide the advantages of gelatin-type sensitization, without the undesirable processing characteristics of the binder itself.

In general the invention comprises a conventionally made emulsion to which has been added a small amount of pyrrolidine, 2-pyrrolidine carboxylic acid (proline), or 4-hydroxy-2-pyrrolidine carboxylic acid (hydroxyproline) to improve its sensitivity to radiation without increasing its fog level. The emulsion may be one of various gelatino-silver halide emulsions and may include those having lower gelatin binder content. The sensitizing agents of this invention should be added in amounts from 0.05 to 5.0 grams per 1.5 mole of silver.

In the preferred process of the invention the pyrrolidine,

## 2

proline, or hydroxyproline is added to the emulsion after digestion and before coating, although it may be added any time after the emulsion is coagulated, washed, and redispersed. The preferred emulsion product of this invention contains from 0.20 to 0.40 gram per 1.5 mole of silver of the pyrrolidine, proline, or hydroxyproline and also contains a reduced amount of gelatin of about 80 grams to 130 grams per 1.5 mole of silver. This will give a photographic element which has a lower binder content and can be processed faster after exposure without a substantial loss in photographic sensitivity. The preferred silver halide is silver bromoiodide.

Several preferred embodiments of the present invention are illustrated by the following examples.

## EXAMPLE 1

A gelatino silver bromoiodide, X-ray emulsion, containing 98.2 mole percent of AgBr and 1.8 mole percent of AgI, sensitized with gold and organic sulfur, and containing approximately 280 grams of gelatin per 1.5 mole of silver was made in the conventional manner. After digestion at 137° F. for 40 minutes and addition of stabilizing and coating aid adjuvants, the emulsion was divided into three parts, with varying amounts of proline being added to each part.

Coated samples were exposed to X-ray radiation through an aluminum  $\sqrt{2}$  stepwedge and no screen, for one minute at 200 kilovolts potential and 4 milliamps current. The samples were exposed, processed, and read as in Example 2, except that the relative speeds were measured at a density of 1.5. The following table shows the sample compositions and the resulting relative speed, average gradient, and net fog levels.

| Sample No. | Amount of Proline (g./1.5 moles of AgBr) | Relative Speed | Average Gradient | Net Fog |
|------------|------------------------------------------|----------------|------------------|---------|
| 1-----     | 0                                        | 673            | 2.66             | 0.16    |
| 2-----     | 0.05                                     | 682            | 2.51             | 0.11    |
| 3-----     | 0.25                                     | 710            | 2.56             | 0.11    |

## EXAMPLE 2

A gelatino silver bromoiodide, X-ray emulsion, containing 98.2 mole percent of AgBr and 1.8 mole percent of AgI, was coagulated, washed, and redispersed by the method described in assignee's patent to J. A. Moede, U.S. 2,772,165. The redispersed emulsion, comprising approximately 105 grams of gelatin per 1.5 mole of silver, was sensitized with gold and sulfur compounds in the conventional manner. After digestion, the emulsion was cooled and dextran added as described in assignee's patent to A. B. Jennings, U.S. 3,063,838. Stabilizers and coating aids, such as saponin, were also added to the emulsion. The emulsion was then divided into two equal parts. To the first part was added 0.32 g./1.5 moles of Ag of 2-pyrrolidine carboxylic acid; to the second part nothing was added.

Two samples, coated on one side, were exposed to X-ray radiation through a medium speed fluorescent medical X-ray screen and an aluminum  $\sqrt{2}$  stepwedge for  $\frac{1}{20}$  second at 70 kilovolts potential and 2 milliamps current. Each sample was developed, fixed, washed, and dried in the conventional manner. In order to simulate double sided coating, each sample was cut longitudinally through the stepwedge exposed area, and the halves of the sample were placed, base sides in contact with each other with steps of equal density matched, in a conventional densitometer. The relative speeds of the two samples were measured at a density of 1.0 and the net fog reading was obtained by subtracting base density from the readings.

The sample with the 2-pyrrolidine carboxylic acid added exhibited higher relative speed, 197, and no increase in

net fog level, 0.16, when compared to the control sample with no 2-pyrrolidine carboxylic acid added (speed, 153; net fog, 0.16).

### EXAMPLE 3

An emulsion was prepared as in Example 2, except that no 2-pyrrolidine carboxylic acid was added. The quantity of emulsion was divided into ten equal parts, into which various quantities of pyrrolidine, 2-pyrrolidine carboxylic acid (proline), and 4-hydroxy-2-pyrrolidine carboxylic acid (hydroxyproline) were added just prior to coating. The table below indicates the composition of the various emulsions and the sensitometric results obtained after exposure and processing as described in Example 2.

| Sample No. | Compound Added      | Amount (g./1.5 moles of Ag) | Relative Speed | Average Gradient | Net Fog |
|------------|---------------------|-----------------------------|----------------|------------------|---------|
| 1.....     | Control.....        | 0                           | 153            | 2.37             | 0.16    |
| 2.....     | Pyrrolidine.....    | 0.05                        | 180            | 2.80             | 0.16    |
| 3.....     | do.....             | 0.10                        | 190            | 2.63             | 0.15    |
| 4.....     | do.....             | 0.20                        | 196            | 2.57             | 0.18    |
| 5.....     | Proline.....        | 0.08                        | 173            | 2.35             | 0.16    |
| 6.....     | do.....             | 0.16                        | 183            | 2.66             | 0.18    |
| 7.....     | do.....             | 0.32                        | 197            | 2.68             | 0.16    |
| 8.....     | Hydroxyproline..... | 0.09                        | 160            | 2.46             | 0.14    |
| 9.....     | do.....             | 0.18                        | 170            | 2.70             | 0.14    |
| 10.....    | do.....             | 0.36                        | 180            | 2.64             | 0.16    |

### EXAMPLE 4

An emulsion was prepared as in Example 2, except that prior to digestion the emulsion was divided into two parts, one part having proline added to it prior to digestion and one part continuing through the digestion step without proline. After digestion, the emulsion containing no proline was divided into two parts, a control and a portion to which proline was added. Coated samples were exposed, processed and analyzed as in Example 2. The compositions and results are shown in the table below.

| Sample No. | Amount of Proline (g./1.5 mole Ag) |                 |                |                  |         |
|------------|------------------------------------|-----------------|----------------|------------------|---------|
|            | Before Digestion                   | After Digestion | Relative Speed | Average Gradient | Net Fog |
| 1.....     | 0                                  | 0               | 139            | 3.22             | 0.23    |
| 2.....     | 0.16                               | 0               | 104            | 3.48             | 0.27    |
| 3.....     | 0                                  | 0.08            | 146            | 3.04             | 0.17    |
| 4.....     | 0                                  | 0.16            | 158            | 3.06             | 0.20    |

### EXAMPLE 5

An emulsion was prepared as in Example 2, except that just after digestion and prior to the addition of final adjuvants, the emulsion was divided into six parts and a different amount of proline was added to each part. The compositions and sensitometric data are shown in the table below, the coated samples being exposed and processed as in Example 2.

| Sample No. | Amount of Proline (g./1.5 moles of Ag) | Relative Speed | Average Gradient | Net Fog |
|------------|----------------------------------------|----------------|------------------|---------|
| 1.....     | 0                                      | 166            | 2.02             | 0.27    |
| 2.....     | 0.20                                   | 181            | 2.06             | 0.21    |
| 3.....     | 0.40                                   | 177            | 2.12             | 0.28    |
| 4.....     | 5.0                                    | 185            | 2.22             | 0.37    |

### EXAMPLE 6

A gelatino silver bromochloride emulsion, containing 80.0 mole percent of AgBr and 20.0 mole percent of silver chloride, was coagulated, washed, and redispersed by the method described in assignee's patent to J. A. Moede, U.S. 2,772,165. The redispersed emulsion, containing bulking gelatin and gold and sulfur sensitizers was digested at 136° F. for 40 minutes. After digestion, stabilizers and coating aids, such as saponin were added, and the resulting emulsion was divided into three portions,

each containing 1.5 moles of silver halide and 100 grams of gelatin. A different amount of proline was added to each portion.

Single coated samples of each emulsion were prepared by methods well known in the coating art, and each sample was exposed through a  $\sqrt{2}$  stepwedge to a xenon flash of  $10^{-4}$  seconds duration at a distance of 6½ inches, developed in a high energy developer, fixed, washed, and dried by conventional methods. The relative speed of each sample was measured at a density of 3.5 by conventional methods on a standard densitometer, as was the average gradient and net fog. The compositions and sensitometric results are shown in the table below:

| Sample No. | Amount of Proline (g./1.5 moles of Ag) | Relative Speed   | Average Gradient | Net Fog |
|------------|----------------------------------------|------------------|------------------|---------|
| 30 1.....  | 0                                      | <sup>1</sup> 100 | 3.00             | .09     |
| 2.....     | 0.40                                   | 115              | 3.00             | .09     |
| 3.....     | 0.80                                   | 124              | 3.10             | .10     |

<sup>1</sup> The speed of the control was assigned the value 100.

35 The embodiments of the invention in which an exclusive property or privilege is claimed are defined as follows:

1. A gelatino-silver halide photographic emulsion containing from about 0.05 to 5.0 grams per 1.5 mole of silver a sensitizer of pyrrolidine, 2-pyrrolidine carboxylic acid or 4-hydroxy-2-pyrrolidine carboxylic acid.

2. An improved emulsion as defined in claim 1 where said emulsion contains about 80 to 130 grams of gelatin per 1.5 mole of silver.

3. An improved emulsion as defined in claim 2 where said sensitizer is present in an amount of about 0.20 to 0.40 gram per 1.5 mole of silver.

4. A gelatino-silver halide photographic element having a gelatino-silver halide emulsion layer containing from about 0.05 to 5.0 grams per 1.5 mole of silver a sensitizer of pyrrolidine, 2-pyrrolidine carboxylic acid or 4-hydroxy-2-pyrrolidine carboxylic acid.

5. An improved photographic element as defined in claim 4 where said element contains about 80 to 130 grams of gelatin per 1.5 mole of silver.

6. An improved element as defined in claim 5 where said sensitizer is present in an amount of about 0.20 to 0.40 gram per 1.5 mole of silver.

7. In a process for preparing a gelatino silver halide the improvement which comprises adding to said emulsion from about 0.05 to 5.0 grams per 1.5 mole of silver a sensitizer of pyrrolidine, 2-pyrrolidine carboxylic acid or 4-hydroxy-2-pyrrolidine carboxylic acid.

### References Cited

#### UNITED STATES PATENTS

2,699,391 1/1955 Mueller ----- 96—107  
2,740,713 4/1956 Warren ----- 96—107

70 NORMAN G. TORCHIN, Primary Examiner

RICHARD E. FICHTER, Assistant Examiner